

## UNITED STATES PATENT OFFICE.

NIELS C. CHRISTENSEN, OF SALT LAKE CITY, UTAH.

## PROCESS OF CONCENTRATING OXIDIZED ORES AND MINERALS.

No Drawing.

Application filed December 14, 1918. Serial No. 268,675.

*To all whom it may concern:*

Be it known that I, NIELS C. CHRISTENSEN, a citizen of the United States, residing at Salt Lake City, in the county of Salt Lake and State of Utah, have invented certain new and useful Improved Processes of Concentrating Oxidized Ores and Minerals, of which the following is a specification.

My process relates to the concentration of oxidized minerals in ores or mixtures of minerals. As is well known to metallurgists no satisfactory process for the concentration of oxidized ores is known at the present time. The ordinary methods of mechanical concentration, such as are successfully used for the concentration of sulphides, do not give commercial results on many oxidized ores. The air-froth flotation process which has revolutionized the concentration of sulphide ores has not been found applicable to the oxidized ores. The hopes entertained by some metallurgists that the sulphidizing, or sulphide filming or coating of lead and copper minerals; i. e., changing them superficially to sulphides, would make possible the treatment of these ores by this process have not been realized. It is thus seen that up to the present time no successful process for the concentration of the oxidized ores and minerals has been invented and it will be appreciated by all who are familiar with mining and metallurgy that a process which will successfully concentrate the oxidized ores, would be a new development in the art and would be of great value and wide application.

By my process the oxidized ores and minerals may be concentrated with the same degree of efficiency that has been attained in the concentration of sulphides.

The process is applicable to the oxidized ores and minerals as such; i. e., the ores require no preliminary chemical treatment such as superficial alteration to sulphides or sulphide filming or coating.

My process is in general applicable to the concentration of the non-silicate oxidized minerals and the separation of these from quartz (and other silica minerals) and silicate gangue minerals and is therefore not generally applicable to ores which contain no quartz or silicates or in which the percentage of these is so small that their removal would not increase the value of the ore sufficiently to justify the operation. In

the specifications I have called those minerals which may be concentrated by my process i. e., the non-silicate minerals, the ore-minerals and the others, i. e., quartz and silicate gangue minerals the gangue-minerals. In some cases, however, a modification of my invention may be used in the treatment of the ores containing no siliceous gangue minerals for the preferential separation of the other minerals.

My process makes use of a selective action by which the non-silicate minerals and some of the silicate ore-minerals are concentrated and separated from the quartz and silicate gangue minerals. This selective action is more or less preferential with regard to the non-silicate minerals and this preferential action may be utilized with some ores consisting mainly of the non-silicate minerals to separate these minerals by a modification of the process as ordinarily applied to ores containing siliceous gangue material.

My process consists of the following steps:

1. The freeing of the different constituent mineral particles of the ore from each other and their reduction to a suitable size.

2. The selective oiling and selective oil-flocculation of the mineral particles to be concentrated, in a pulp made by mixing the comminuted ore with water.

3. The levitation of the oil-mineral flocules by the incorporation therewith of fine bubbles of a suitable gaseous medium, thus forming buoyant oil-mineral-bubble flocules.

4. The separation of these oil-mineral-bubble flocules from the remainder of the pulp.

The process is carried out as follows:

The ore is first crushed to free the different minerals and ground to the desired mesh; the comminuted ore is then mixed with water to form a pulp; sufficient of a suitable oil or oily compound is added and thoroughly mixed with the pulp in such a manner as to subdivide the oil into a large number of relatively very small particles and to distribute these throughout the pulp. This results in the selective oiling and selective oil-flocculation of the minerals to be concentrated. Preferably at the same time that the oil is thus being distributed through the pulp a large number of small air bubbles, or bubbles of other inert gas, are injected into the pulp and thoroughly mixed therewith.

During the injection of the air bubbles the pulp is thoroughly agitated and mixed. The subdivision of the oil and injection of the air bubbles and their admixture with the pulp are preferably conducted simultaneously but the oil may be mixed with the water before the addition of the ore or may be mixed with the pulp during the grinding operation. The result of the admixture of the fine air bubbles with the pulp is that some of these become incorporated in and attached to the oil-mineral floccules and levitate these and render them buoyant, forming an oil-mineral-bubble floccule. After the formation of the oil-mineral-bubble floccule the pulp is allowed to become sufficiently quiescent so that the oil-mineral-bubble floccules rise to the surface of the pulp. The mass of buoyant oil-mineral-bubble floccules thus formed at the surface of the pulp is then removed, leaving the particles of quartz and silicate gangue minerals in the pulp.

The foregoing is only a general statement of the manner of carrying out the process without reference to the details of each step, which are given in the following:

1. *Freeing of the different mineral particles and grinding of the minerals to be concentrated to a suitable fineness.*

The proper carrying out of this step is very important. It is obvious that the ore must be crushed to such a size that the different mineral constituents are freed from each other, otherwise no separation could be made. The minerals to be concentrated must also be ground sufficiently fine to be amenable to the process, in most cases to 80 mesh or finer. The fine grinding of the ore must not be done with iron (i. e. iron or steel) grinding parts unless the effect of this grinding is removed before the concentration treatment, as the quartz or silicate gangue-minerals thus finely ground flocculate with the ore-minerals to be concentrated and the selective action of the oil flocculation is thus destroyed. This effect is more pronounced the finer the grinding, the longer the time of grinding, the softer the grinding media and the harder the gangue mineral. This effect when grinding is done with cast iron balls is more pronounced than with manganoid balls, and if the gangue is mostly soft mica, the effect is relatively slight. That it is essential that fine grinding of the ore be not done with iron or steel grinding media, unless the effect is removed as later described, is readily seen from the following examples: A siliceous oxidized lead ore containing 65%  $\text{SiO}_2$  and 10% lead finely ground in a pebble mill gave a concentrate carrying 95% of the lead and only 10% silica. The same ore ground to the same mesh and even to a much coarser mesh, with iron balls gave no concentration whatever,

the whole of the ore oil-flocculated and there was no selective action. An oxidized copper sandstone ore carrying 12% copper, finely ground in a pebble mill gave a concentrate carrying 98% of the copper in the ore and assaying 48% copper and 12.5% silica and a tailing assaying only 0.3% Cu. This ore ground to 100 mesh with steel balls gave no concentration whatever, the whole of the ore oil-flocculated and there was no selective action and no separation. The same ore ground in a ball mill for only 15 minutes and to a much coarser mesh gave a concentrate assaying 17.5% copper and 66.4%  $\text{SiO}_2$  weighing 60% of the ore, a middling assaying 4.5% Cu, weighing 16% of the ore and a tailing assaying 2.5% Cu weighing 24% of the ore, which shows practically no concentration and gave results which are worthless from a commercial standpoint.

Ores finely ground on an iron bucking board or in the ordinary iron disk grinder give no concentration whatever as the whole of the ore oil-flocculates and there is no selective action when treated by my process.

In practical operation the fine grinding should preferably be done with a pebble mill unless the effect of grinding with iron is removed before the treatment as later described. All metallic iron mixed with the ore, from the mining operation, should be preferably removed before fine grinding in order to secure the best results.

For laboratory tests the fine grinding should be done in a porcelain pebble mill with quartz pebbles or with a porcelain mortar and pestle. Iron from the coarse crushing should preferably be removed before the fine grinding to secure the best results.

The effect on the finely ground quartz and silicate gangue minerals of contact with metallic iron, while the pulp is in vigorous movement so as to scour metallic iron, is also very detrimental, as this causes the quartz and gangue silicates to oil flocculate in my process and prevents their separation from the non-silicate minerals.

This may be simply demonstrated in the following manner: The finely ground quartz is mixed with water and shaken in a test tube for one minute with finely divided clean particles of metallic iron and the metallic iron then removed from the pulp with a magnet; upon the addition of the oily agent and shaking the test tube vigorously,

all the silica oil-flocculates and the floccules are levitated in a manner similar to the non-silicate minerals. The same result is also secured by the similar treatment of feldspar and other silicate gangue minerals.

The fine gangue minerals thus treated also oil-flocculate preferentially with regard to the ore-minerals. If the finely ground gangue minerals are shaken with water in a clean iron pipe for three minutes and then transferred to a test tube and the oily flo-

120  
125  
130

culating agent added and the test tube shaken vigorously so as to violently agitate the mixture, all the fine silica oil-flocculates and the floccules are levitated and come to the surface of the pulp when the shaking ceases, in a manner similar to the non-silicate minerals. If very finely ground metallic iron, in any considerable percentage is mixed with finely ground ore, the result is the total oil-flocculation of the ore. If only a very small amount of iron is used the entire mass may not oil-flocculate but the floccules carry more gangue minerals than they otherwise would, the effect being proportional to the amount of metallic iron in the pulp. A similar effect results when very fine metallic aluminum, copper or lead are added to the ore pulp, but the effect is not nearly so strong as with iron and is less with lead than with aluminum or copper. The theory of the action of these metals is given later. This effect is relatively slight and of very little importance as compared with the effect of the iron. Quartz and silicate minerals, alone, when finely ground on an iron bucking board or in an iron disc pulverizer, or in a ball (iron or steel balls) mill are entirely oil-flocculated and the floccules levitated in a manner similar to the non-silicate minerals. From the foregoing it is seen that it is essential that the fine grinding of ores preparatory to treatment by my process must not be done with metallic grinding media, as this destroys the selective action of my process and prevents the concentration of the ore minerals and their separation from the siliceous gangue minerals. As it is the object of my process to concentrate the non-silicate minerals and separate them from the quartz and siliceous gangue minerals in the ore, and since grinding with iron causes the quartz and silicate gangue minerals to oil-flocculate and levitate in my process in a manner similar to the non-silicate minerals and therefore destroys the selective action of my process and prevents the separation of these two classes of minerals by my process, it is obvious that the fine grinding of ores to be treated by my process must not be done with iron grinding media, unless the effect of this grinding is removed by a special treatment before applying my process. It is best that the ground ore be not kept long in contact with metallic iron or iron pumps or pipes before being concentrated, as this also tends to destroy the selective action of my process by causing the quartz and silicate gangue minerals to flocculate in a manner similar to the non-silicate minerals. The effect of grinding or scouring with metallic iron may be entirely removed by the addition of a very small amount of acid, e. g.  $H_2SO_4$ , to the ground ore and agitating the pulp and

then entirely neutralizing the acid with lime-stone previous to concentration. Obviously this could not be done commercially if the ore contained much calcite. The neutralizing should not be done with an alkali, however, as the ore thus treated will still non-selectively oil-flocculate to a considerable extent. A theory explaining the effect of the iron is given later. Relatively fine grinding of the minerals to be concentrated is necessary to successful oil-flocculation and concentration. The fineness varies with the mineral, for instance, carnotite must be ground to extreme fineness to get a good recovery, while calcite may be much coarser. In general most of the minerals to be flocculated should be 80 mesh or finer.

2. *The selective oiling and selective oil-flocculation of the minerals to be concentrated.*

This and the following step, which are preferably combined in one operation in actual practice, are the main parts of my process. In order that the process operate successfully, it is essential that this step be properly carried out.

First—the right kind of oils must be used. Only those oils or oily compounds can be used which not only selectively oil the non-silicate (and also the silicate ore minerals) but also bring about the selective-oil-flocculation of these minerals.

The pure volatile or essential oils alone, i. e. without admixture with other oils or resins (and excepting rosin or colophony which is sometimes classed with these oils but is not an essential oil) are useless in my process, as they do not selectively flocculate the non-silicate minerals. The slight flocculating action shown when a large excess of these oils is used is very probably due to rosin acids remaining in the oil. The refined or steam distilled pine oils, terpenes, turpentine and other related and similar oils must be used in very large excess to show any flocculating effect. The crude pine oils and turpentine which contain more rosin acids show a slightly greater flocculating effect. Rosin spirits, which contain still more rosin acids, gives fair results. Rosin oils, containing a considerable percentage of rosin acids, give fairly good results. Rosin or colophony, which consists largely of free rosin acids (mainly abietic acid) dissolved in essential oils so that the mixture contains a large percentage of rosin gives fairly good results. To secure the best results, however, it is preferable not to use any of the essential or partially soluble oils in the flocculation medium as they tend to prevent the selective oiling and flocculation of the ore minerals.

The mineral oils alone (i. e. without ad-

mixture with other oils or resins) are useless in my process as they do not selectively oil-flocculate the ore-minerals. When used in very large excess a slight flocculating effect 5 may be shown, but this is probably due to small amounts of fixed organic oils contained in the mineral oil in the form of dissolved bitumen waxes which contain free fatty acids. By mineral oils is meant the 10 petroleum oils, shale oils, coal tar oils and creosotes, lignite tar oil, etc. etc.

Rosin dissolved in the mineral oils so that the oily compound or mixture contains a large percentage of rosin gives very good 15 results.

The fixed oils as a class give excellent results. Of the animal oils, the fish oils such as menhaden oil, salmon oil, etc. give excellent results; the liver oils, such as cod liver 20 give good results; the blubber oils such as whale oil give good results. The animal fats such as tallow dissolved in other oils give good results, and the animal waxes such as sperm oil give excellent results. Among 25 the vegetable oils, a large number of drying, semi-drying and non-drying oils, such as linseed oil, castor oil, olive oil, etc., give good results. The vegetable fats such as cocoanut oil and palm oil give good results.

30 The liquid fatty acids such as oleic acid give excellent results. The solid fatty acids such as stearic in solvents which will dissolve a large percentage of the acid give good results.

35 From the foregoing it is seen that an extremely large number of combinations of oils may be useful in my process but as will be seen also from the foregoing there is one essential feature in all oils that can be successfully used in my process and that is that the oil or oily compound must contain a proportion of a fatty acid or rosin acid, either free or combined, or some other analogous compound which acts in a similar 40 manner. It should here be noted, as bearing on the theory later given, that the fatty acids combined with inorganic bases (other than the alkalies) form insoluble "metallic soaps" and that rosin combines with these 45 bases to form the so-called rosin greases. It should also be noted that the suitable oils are insoluble in water and also that they break up into minute globules when vigorously shaken with water.

50 In practice I have secured the best results with oleic acid, menhaden oil, and rosin dissolved in kerosene or one of the coal tar oils. Each ore should, however, be tested to see which oil or oily compound 55 gives the best results in its concentration as some oils give better results with certain ores than do other oils.

The second feature of importance is the amount of oil necessary. The amount of oil necessary to secure certain results is fairly

sharply defined. In general up to a certain limit the amount of quartz or silicate gangue material carried up by the floccules is inversely proportional to the amount of oil used. This limit is slightly over 10 per cent (10 to 15 per cent) of the weight of the minerals to be concentrated. For example, if 20 per cent of the weight of the ore is concentrate, the amount of oil used should be slightly over 2 per cent of the weight of 75 the ore.

When only a small proportion of the ore is to be concentrated this proportion of oil must usually be increased somewhat. The effect of the varying amount of oil on the 80 percentage of quartz or silicate gangue-minerals carried by the floccules is shown in the following examples: An oxidized lead ore carrying 33 per cent non-silicate minerals and 67 per cent quartz gave in each 85 case cited below approximately the same recovery (approximately 95 per cent) of the non-silicate minerals in the concentrates, but with 1½ per cent menhaden oil (1½ per cent of the weight of the ore) the floccule-concentrates carried 30 per cent silica; with 2 per cent oil, 25 per cent silica; with 2½ per cent oil, 20 per cent silica; with 3 per cent oil, 15 per cent silica; with 3.5 per cent oil, 12 per cent silica; 4 per cent oil, 10 per cent silica; 4½ per cent oil, 9 per cent silica. A manganese ore (manganite in a porphyry gangue) carrying 50 per cent manganite and the remainder feldspar, gave approximately 90 a 93 per cent recovery in all the concentrates; but with 2 per cent oil the concentrates carried 20 per cent insoluble; with 3 per cent oil, 14 per cent insoluble; with 4 per cent oil, 10 per cent insoluble; with 5 per cent oil 7.5 per cent insoluble; with 6 per cent oil, 6 per cent insoluble. Tests on oxidized copper ores in sandstone gave similar results. In a general way it may be stated that the best concentration is secured by using a weight of oil equal to between 10 and 15 100 per cent of the weight of concentrates. More oil than this gives very little improvement in the grade of concentrates. Considerable more oil may be used without 105 detrimental effect, but if a very large excess of oil is used the floccules may lose their buoyancy to a very marked degree and be difficult to levitate and remove from the pulp. This is more pronounced with the 110 heavier minerals, such as anglesite and cerusite, etc., than with the lighter minerals. This percentage of oil should be figured on the active oil in any oily compound and not on the total of the mineral oils or other oils used as solvents plus the active ingredients 115 (such as resin) e. g. in a rosin-kerosene mixture the percentage of oil should be figured on the rosin content alone if the mixture is dilute with regard to the rosin.

The foregoing is of course only a general 120

statement of the amount of oil to be used. The absolute amount necessary to secure the best results is greater, the finer the grinding, very slightly greater with dilute pulps and less with warm than with cold pulps. Different ores also require somewhat different proportions of oil to secure similar results.

The character of the floccules also varies progressively with the increasing proportion of oil. With the small proportion of oil the floccules are lighter, less discrete and carry more fine air bubbles (when levitated) and more siliceous gangue-material and do not maintain their flocculate character so distinctly after being removed from the pulp. With increasing proportions of oil the floccules become progressively heavier, more discrete, carry fewer fine air bubbles and less siliceous gangue-material, and maintain 20 their flocculate character distinctly after separation from the pulp.

The manner of bringing the oil into contact with the mineral particles is important. The oil must be broken into minute globules in the pulp in order to act well in selectively oiling and oil-flocculating the ore-minerals. This may be brought about by mixing the oil with the pulp during the grinding operation but is preferably done by a very vigorous mechanical agitation of the oil or oily compound mixed with the pulp containing the comminuted ore. By this operation the particles of the ore minerals are selectively oiled and flocculated; i. e., brought together in small clinging aggregates. The size of these aggregates will vary with different minerals and the fineness of grinding. The floccules of the more readily oil-flocculable minerals are usually larger, as large as  $\frac{1}{8}$ " in average diameter, the less readily oil-flocculable minerals which require fine grinding may be much smaller. These aggregates contain the minerals to be concentrated (i. e. the ore-minerals) and also practically all the oil added to the pulp (unless some essential or partially soluble oil is used which is not desirable) and a small amount of gangue-mineral. The oil may be recovered from the concentrates by suitable methods such as dissolving with suitable solvents and distilling off the solvents, and may be used again in the process. This step of oiling and flocculating is preferably carried out at the same time that the floccules are levitated; the selective oiling and flocculation and levitation being all carried out in one operation.

### 3. The levitation of the oil floccules.

The levitation of the oil floccules is brought about by the injection of numerous fine gas bubbles (preferably air) into the pulp and thoroughly mixing them therewith. In order to secure good results the bubbles must be relatively very small. Any relatively large bubbles have very little effect in the levita-

tion of the floccules. This levitation may be brought about by mechanically mixing or beating air into the pulp with paddles or by projecting air bubbles through a porous medium into the pulp, or by a combination of these two methods. The best results are obtained by the mechanical or combined methods as it is difficult to secure fine enough bubbles by passing the gas through any ordinary porous media now used. As previously stated the selective oiling and selective oil-flocculation and the levitation of the oil-floccules are all best brought about in the same operation, preferably by the vigorous mechanical agitation of the pulp in such a manner as to break up the oil into fine globules and inject numerous fine air bubbles into the pulp and thoroughly mix these and the mineral particles in the pulp. By this operation many fine bubbles become incorporated in and attached to the oil-mineral floccules, forming a buoyant oil-mineral-bubble floccule. If as is preferred the selective oiling, oil-flocculation and levitation are all performed in a single operation, the oil-mineral-bubble floccules are formed at once and may be removed as described in the next step. I have found that the machines which give best results are those which furnish the largest supply of the finest bubbles during the operation.

In the foregoing I have made no statement as to the kind of solution in which this process of oil-flocculation should be carried out. This is a vital feature of the process. In general, my process will not operate successfully with acid or alkaline solutions in the pulp and gives much better results when the solution is free from dissolved salts which act as flocculating agents.

Mineral acids, even in a very small amount entirely prevent the oil-flocculation of the ore-minerals. For example, with many ores as little as .025 per cent of free  $H_2SO_4$  in the solution entirely prevents the oil-flocculation. Most ores contain sufficient calcite or other soluble material to neutralize small quantities of acid in the solution, so that in operating the process the solutions must be tested for free acid. If the solution in the pulp is clearly acid to litmus the ore-minerals cannot be successfully oil-flocculated. After the ore-minerals have been completely oil-flocculated the acid de-flocculates them with difficulty and the acid is therefore much less injurious after the flocculation. The effect of the acid after oil-flocculation is to cause the oil-mineral-bubble floccules to contract somewhat and become more dense and to lose a part of the air bubbles which makes them more difficult to levitate and separate from the pulp. In some cases in which the concentrates contain much carbonate the presence of the acid may be very injurious even after the oil-flocculation. If

the solution contains  $H_2SO_4$  previous to flocculation, the acid may be neutralized with  $CaCO_3$  and the ore-minerals can then be oil-flocculated and concentrated.

5 Free alkali, even in very small amount in the water, also prevents the oil-flocculation of the ore-minerals. For example, as little as .01%  $NaOH$  completely prevents oil-flocculation and gives a white soapy foam.

10 Some ores contain material which will neutralize the  $NaOH$  and others have the power of absorbing the  $NaOH$  so that it is necessary to test the solution. If the solution in the pulp is clearly alkaline to litmus paper

15 the ore minerals cannot be oil-flocculated in this solution. The alkali in the pulp may be neutralized with acid and its effect destroyed and the ore-minerals can then be oil-flocculated. If the alkali is added after the oil-flocculation, it destroys the levity of the oil-mineral-bubble floccules and causes them to sink and with continued agitation deflocculates them. Soap, which is alkaline, even in small quantity also prevents the oil-flocculation

20 and destroys the levity of the floccules already formed.

Salts, such as  $NaCl$ , which act as ordinary flocculating agents are not so objectionable as the acids or alkalis but it is very much preferable that they be absent. The effect of these salts is to first cause the non-selective oil-flocculation of all the minerals in the pulp similar to the metallic iron, but with continued vigorous agitation the oil-flocculation becomes more selective and the particles of gangue-minerals are rejected by the floccules. This makes it necessary, in order to secure any concentration with salts in solution, that the pulp be subjected to vigorous agitation for a period long enough to make the non-selective oil-flocculation selective before the removal of the concentrates. This is objectionable in any commercial operation, also the concentrates are not so clean as without the salts. It is therefore preferable that no salts be present in the solution. This effect is less pronounced with ores having a small percentage of concentratable minerals than with those having a larger percentage. Common salt in as small a proportion as .04% in the solution will give these effects. The gangue-minerals show no oil-flocculation whatever with salt in the pulp unless some ore-minerals are also present in the pulp. Salts which are hydrolyzed in solution give effects intermediate between the acids or alkalis and the neutral salts, the precise effect depending on the degree of hydrolysis and nature of the ore. Though the gangue-minerals alone show no oil-flocculation with the salts in solution when the pulp becomes quiet the particles of gangue-minerals do flocculate in the ordinary manner and the flocks slowly settle just as in the ordinary

and well known process of flocculation and sedimentation or settling. If the ore-minerals are first oil-flocculated and levitated and removed from the pulp and salt added to the remaining pulp the gangue flocculates in the ordinary manner and the flocks settle in precisely the same manner as in the previous case. These and other phenomena show that the two kinds of flocculation are entirely independent phenomena.

I have used the term "flocks" in referring to the product of ordinary flocculation, and floccule in referring to oil-flocculation in order to distinguish between the two as they are entirely dissimilar in their characteristics. The ordinary flocks cannot be levitated; the oil-floccules are readily levitated, i. e., made into oil-mineral-bubble floccules; the ordinary flocculation is non-selective; the oil-flocculation is selective; the ordinary flocculation is relatively slow; the oil-flocculation is very rapid; the ordinary flocks are easily broken up and dispersed; the oil-floccules are relatively permanent and maintain their character well; the ordinary flock is relatively much more dispersed than the oil-floccule and settles much more slowly than the delevitated oil-floccule.

My process is also preferably carried out in relatively dilute pulps; i. e., over six and up to fifteen or more of water to one of ore. The finer the grinding the more dilute the pulp should be to secure good results. Warm pulps give slightly better results than cold pulps.

My process should also not be carried out in direct contact with the metal of an iron machine, as good results cannot be secured. The effect of the violent agitation of the oil and pulp with the metallic iron is to oil-flocculate a large part of the fine gangue particles as previously described and to more or less destroy the selective action of the process. Slightly better results can also be secured in a glass or wooden machine than in a metallic machine, such, for example, as one made of aluminum.

#### 4. The separation of the levitated floccules or oil-mineral-bubble floccules.

The last step, the separation of the levitated floccules or oil-mineral-bubble floccules, is brought about by allowing previously agitated pulp to come to a relatively quiescent condition so that the buoyant oil-mineral-bubble floccules may come to the surface of the pulp. The mass of buoyant floccules thus formed, may then be skimmed off the surface of the water by mechanical means, or allowed to accumulate until they reach a depth sufficient to cause them to overflow over an edge of the vessel (which should be very slightly higher than the level of the pulp). Though the oil-mineral-bubble floccules are sufficiently buoyant to

be readily removed in this manner, a slightly better grade of concentrate can be secured if a number of fine bubbles are injected into the pulp during this part of the process.

- 5 If large bubbles are injected into the pulp in this stage of the process they may serve to drive the levitated floccules over the discharge lip of the apparatus but this action is merely a mechanical means of removing  
 10 the floccules and has no real relation to the process itself. If many large bubbles occur at this stage of the process it has been found to be disadvantageous rather than helpful as the pulp is thereby kept in constant agitation  
 15 which interferes with the rising of the floccules and also disturbs the mass of these at the surface by constantly breaking through the mass and keeping it in agitation. Also it is perfectly obvious that the  
 20 ore-minerals may first be selectively concentrated into oil-mineral-bubble floccules and then be allowed to lose their bubbles and settle as less buoyant oil-mineral floccules and these can then be separated from  
 25 the remainder of the pulp by any suitable washing or concentrating process and machinery of the same kind as those now in general use in the ordinary mechanical concentration of sulphide minerals, but this is  
 30 not a preferred method, though it can be used and will give good results in many cases.

In the treatment of most ores the concentrating operation is preferably divided into  
 35 two steps. An oil-mineral-bubble floccule-concentrate is first separated from the remainder of the ore as described. This concentrate is then retreated or cleaned by a similar operation to remove as much more  
 40 of the gangue material as possible. All the oil used may be added in the first, or "roughing" operation and the second, or "cleaning" operation be conducted with the addition of more oil, but it is much preferable  
 45 in the majority of cases to add most (say three-fourths) of the oil or oily compound in the "roughing" operation, thus forming relatively lighter floccules, and then add the remainder of the oil in the  
 50 "cleaning" operation, forming a heavier floccule. Too light a floccule should not be made in the roughing operation however, as if this is done entirely too much siliceous  
 55 gangue material will be included in the floccules.

The oil-mineral-bubble floccules quickly lose most of the air bubbles when removed from the pulp and dropped into water, and the oil-mineral floccules settle very quickly.  
 60 These oil-mineral floccules maintain their flocculate character with great persistency when sufficient oil has been used, and the removal of the excess water from the floccule-concentrates by filtration is accomplished without difficulty no matter how

fine the grinding. After the removal of the concentrates and settling in water, some of the fine silica included in the floccules gradually separates out and can be removed by washing if desired.

The process may be carried out in any suitable apparatus which will thoroughly agitate the pulp in such a manner as to break up the oil into minute globules and inject or beat air into the pulp in fine bubbles and thoroughly mix these with the pulp and thereafter allow the so-treated pulp to remain in a sufficiently quiescent condition for a long enough period that the levitated floccules come to the surface, so that they can be removed and separated from the remainder of the pulp. Many different types and forms of machines may be used for this purpose and I therefore do not desire to connect the process with any particular machine.

For testing purposes a machine which is intermittent in operation and which uses only one compartment both for the agitation of the pulp and (by stopping the agitation and allowing the pulp to become quiet and the floccules to come to the surface) the separation of the pulp may be used. It is preferable, however, to use a continuous machine of two compartments, one in which the oil-mineral-bubble flocculation is brought about by vigorous agitation and another in which the so treated pulp is allowed to come to a relatively quiet condition so that the buoyant floccules may come to the surface of the pulp and be removed, the two compartments being connected so that there is a constant flow of pulp from the agitation compartment into the separation compartment and back into the agitation compartment in a closed circuit. For commercial operations the latter type of machine would probably be the only type used.

From the foregoing it is clear that the essential feature of the process is the selective concentration of non-siliceous ore-mineral particles in an aqueous pulp into buoyant oil-mineral-bubble floccules and their separation from the remainder of the pulp, which contains the siliceous gangue minerals in a dispersed condition. In order to accomplish this and to secure an efficient concentration it is seemingly necessary:

1. That the minerals to be concentrated be ground relatively fine.
2. That the ore, especially the gangue-mineral, be not finely ground with metallic iron grinding parts, or if so ground that the effect so produced be removed before treatment by the process.
3. That the oil or oily compound used contain a proportion of a fatty or rosin acid or similar compound either free or combined in an oil.

4. That the oil or oily compound be used in sufficient quantities to prevent the carrying of much of the siliceous gangue-minerals into the concentrates, an approximate 5 minimum amount equal to 10 per cent, more or less, of the weight of the concentrates.
5. That the agitation of the pulp be violent enough to break up the oil and air into minute globules and thoroughly mix them 10 with the pulp.
6. That the oil-flocculation be not conducted in an acid or alkaline solution.
7. That the ore be not agitated in contact with metallic iron for any considerable 15 period previous to, or while the oil-flocculation is taking place.
8. That the pulp be brought to a state of sufficient quiescence after the formation of the oil-mineral-bubble floccules that they 20 may come to the surface of the pulp and be removed.
- And to secure the best results it is preferred:
1. That the water in the pulp contain no 25 dissolved electrolytes.
  2. That the oil-flocculation be not conducted with a metallic agitating device.
  3. That essential oils be not used in considerable amount.
- 30 Having described the process, the action of the different minerals is described in the following: As before noted, according to their action in my process, the oxidized minerals are separable into two broad classes.
- 35 Class I. Minerals which cannot be oil-flocculated but remain in a dispersed condition in the pulp, and Class II, minerals which can be oil-flocculated and which may be removed from a pulp by formation of 40 buoyant oil-mineral-bubble floccules as described. To Class I belong all the quartz minerals and all the silicate minerals (except those mentioned in Class II). These are called the gangue-minerals in the specifications and claims. To Class II belong 45 all the non-silicate oxidized minerals and a few silicates such as rhodonite, willemite, garnierite, serpentine talc, etc. These are called the ore-minerals in the specifications and claims. Intermediate between the two main classes are a few silicates, which show 50 a slight degree of oil-flocculation, such as some garnets and chrysolites and prehnite and sodalite. Fortunately, for the value 55 of the process the important gangue-minerals are distinctly of the Class I type and the important ore-minerals of the Class II type, and the intermediate class between the two contains very few minerals of any importance or of frequent occurrence in any considerable percentage in ores. It is of some 60 theoretical interest to note that in general the minerals of Class I are the primary minerals and metamorphic minerals which 65 are formed under conditions of relatively

extreme heat and pressure and the minerals of Class II are the non-silicate and silicate minerals which may be and are usually formed by the action of or precipitation from aqueous solutions at ordinary temperatures and some silicates formed by the complete alteration of some of the minerals of Class I by aqueous solutions, and that the small intermediate class consists of minerals formed by conditions intermediate between the two or by the partial alteration of some of the minerals of Class I. 70

It is also of considerable theoretical importance to note that the minerals of Class I are in general very slightly or slowly 80 acted upon by ordinary chemical reagents, and that the minerals of Class II are in general very easily soluble or readily acted upon by these reagents.

The oil-flocculating effect and oil-floccule levitation effect vary considerably with different minerals of Class II. In general the carbonates, sulphates, phosphates, halides arsenates and chromates, etc. (i. e. chemical salts) oil-flocculate more quickly 90 and the floccules levitate more readily than the oxides or hydroxides, and the latter oil-flocculate more quickly and the floccules levitate more readily than the silicates of this class. Minerals of the same class also 95 exhibit considerable difference in this respect, for example, azurite oil-flocculates more readily and levitates more quickly than malachite, manganite and bauxite oil-flocculate more quickly and the floccules 100 levitate more readily than is the case with hematite and limonite, and rhodonite oil-flocculates and the floccules levitate more quickly than garnierite. This fact makes possible the preferential separation of some 105 of the ore-minerals with a greater or less degree of perfection by the process. For example, in the treatment of an oxidized copper sandstone ore, the first part of the concentrates removed from the pulp was 110 mainly azurite and the last part mainly malachite.

The foregoing statements regarding the action of the oxidized minerals in my process are based on a great number of tests 115 on specimens of all but the rarest minerals and upon samples of numerous oxidized ores of many different kinds.

Sulphide minerals such as galena, etc., act in a manner entirely different to the oxidized ore minerals in my process. For example, if the oil is added during the grinding of an ore containing galena, the galena granulates or coagulates and forms heavy balls, lumps, or granules, which may be separated from the pulp by screening, or by treatment in a classifier or on a concentrating table but cannot be separated by my process; the oxidized non-silicate minerals form buoyant floccules and come to the surface of the pulp 125 130

as previously described but the sulphide granules or balls sink and are left behind with the quartz and silicates in the remaining pulp. If the oil is added to this ore pulp in the levitation machine, in the proportion required in my process, the galena granulates, i. e., forms small lumps or balls, and sinks, while the oxidized ore-minerals form oil-floccules and levitate as previously described.

If the ore contains only a small amount of sulphide minerals as compared with the oxidized ore-minerals, the granulation of the sulphides is somewhat hindered owing to the sulphides being diluted with such a large proportion of oxidized ore minerals, and some of the sulphides will be carried up in the floccules, but my process is not applicable to the concentration of sulphide minerals as such and if the ore contain any considerable quantity of these they must be separated by some other process in order to make a good concentration.

A theoretical explanation of the operation of my process as it appears to be, is as follows, though, of course, it is to be understood that the phenomena which occur are not always readily explainable. Suffice it to say that if the process is carried out as above outlined the results set forth and claimed are effected.

According to this theory three different kinds of forces are active in the process. They are chemical, electrical and physical, and all act more or less in conjunction in all the steps of the process. The electrical part of the theory is that by the agitation of the pulp the different particles of ore, oil and bubbles are electrically charged in the following manner: the silicious gangue-minerals, the oil particles and the air bubbles are all negatively charged; the ore-minerals are positively charged. According to this theory in order for any action to take place all of these particles must be relatively small, otherwise the electric attractions and repulsions of the electrical charges would have little effect, since if the mineral particles are too large the weight of the particles would be so large in comparison to the force of the charge, which resides only on the surface of the particles, that the latter would be unable to act efficiently. The same would be true of the air bubbles and oil globules, since if they are too large the levity of the bubbles or oil globules would be so great as compared with the force of the charge on the surface that these would be unable to act efficiently. Especially the relatively weak attraction of the floccules for the air-bubbles would have no power to hold a large bubble whose buoyant force would be much larger than the attraction of the electrical charges. This explains why large bubbles are not

useful in the process and also explains the losing of the bubbles by the floccules when the fine bubbles coalesce and form larger ones due to the surface tension of the water surrounding the bubbles, which phenomenon is shown by a mass of floccules which is allowed to remain on the surface of the pulp for some time. The electrical part of the theory enters into each step of the process, the chemical into the effect of the iron and the selective action of the oil, and the physical into formation and maintenance of the oil-floccules.

The explanation of the action as a whole is as follows: The positively charged particles of the ore-minerals attract the negatively charged minute globules of oil and the fine air bubbles and the silicious gangue particles. The oil particles wet or oil the particles of ore-mineral, and these two cannot therefore be afterward separated. The negative charge of the oil only partially neutralizes the positive charge of the ore-mineral particle and the residual charge remains on the surface of the particles and its dissipation is prevented by the non-conducting covering of oil. The oiled mineral particle, therefore, still attracts the particles of the gangue-mineral and the fine air bubbles until the effect of the positive charge is neutralized. As soon as this occurs there is nothing to counteract the action of ordinary mass attraction between these particles, and they immediately come together and form floccules. At this stage the floccules are made up of the oiled ore-mineral particles and enough of the gangue particles and fine air bubbles to neutralize the effect of remaining positive charge of the oil-mineral particles. As more oil globules come in contact with the floccules, they are taken up by the oil on the oil-mineral particle, due to the relatively strong action of the surface tension of the oil. The addition of this added amount of oil makes the resultant charge of the floccule negative and tends to disperse it. The result is that some of either the gangue particles or the air bubbles must be rejected as the surface tension of the oil holds the oil wetted ore-mineral particles together.

As the weight of the gangue particles in proportion to the charge carried is much greater than the weight of the air bubbles in proportion to the charge they carry, the result is that the gangue particles are selectively rejected from the floccules. As more oil globules are taken up by the floccules, this selective rejection of the gangue particles continues and the floccules become lighter and more coherent.

As the amount of oil in the floccules still increases, it is found that the rejection of the gangue minerals gradually diminishes and finally reaches a minimum limit. This phe-

70

75

80

85

90

95

100

105

110

115

120

125

130

nomenon of the progressive selective rejection of the gangue-minerals from the floccules can be seen with remarkable clearness by treating a small portion of the low 5 grade oil-mineral floccules from a larger operation, in a test tube partially filled with water. By adding additional oily agent drop by drop, and shaking the test tube vigorously the rejection of the gangue-minerals and their dispersion in the water 10 is made plainly visible. The fact that all the silica cannot be rejected is probably due to the fact that the floccule cannot contain or hold enough of the fine air bubbles to 15 neutralize its residual positive charge and this remaining part is neutralized by the floccule taking up silica. If, however, the floccules are removed from the presence of the gangue-minerals in the pulp and the 20 operation repeated with an excess of fine bubbles present, more of the gangue minerals can be rejected. Also if an excess of fine bubbles is injected into the relatively quiescent pulp during the separation of the 25 floccules from the pulp, more of the gangue particles may be replaced by air bubbles. But as the floccules cannot hold enough fine air bubbles to neutralize the residual positive charge, it is theoretically impossible 30 to displace all of the gangue particles. As more oil is added, the residual positive charge of the floccule becomes less and less until the number of air bubbles it can hold becomes progressively smaller and the floccules lose buoyancy, and with a large excess of oil may lose their buoyancy entirely. 35 Accordingly to this theory also, if the oil-mineral-bubble floccules should be gradually neutralized, i. e. lose the residual positive charge on the ore-mineral by any means 40 after removal from the pulp, they would tend to become dispersed and the gangue particles would be gradually rejected. This does occur when the floccules are removed 45 from the pulp and settled in water. Most of the bubbles are lost almost immediately and the silica is gradually dropped. As the discharge of the residual positive charge on the ore mineral continues (probably by 50 leakage through the oil covering) by the long standing in water, the floccules gradually becomes dispersed but this change is resisted by the oil, the surface tension of which tends to hold the oiled minerals together. As noted in the description of the 55 operation of the process, this does actually take place in practice.

The foregoing description of the method of formation of the oil-floccules explains the great difference in characteristics between the flocks of ordinary flocculation and sedimentation and the oil floccules. The ordinary flocks are held together only by the 60 very weak force of mass attraction (gravity) and these flocks are therefore very easily

broken and very loosely held together. The oil flocks are held together not only by this force but by the much stronger forces of the electrical charges and surface tension of the oil. 70

From the above theoretical consideration there should be a rather indefinite theoretical minimum amount of oil for good work and a rather indefinite theoretical amount above which the addition of oil does no good, 75 and with increasing proportions does harm. The amount of oil used should also theoretically be proportional to the percentage of ore-minerals in the mineral mixture, and should increase somewhat with the fineness 80 of grinding (due to increased surface) and vary with the differing charges carried by different kinds of minerals. The foregoing theoretical requirements are strikingly met by the following facts observed in the practical operation of the process. 85

1. That the amount of quartz and silicates in the floccules progressively decreases as the oil is increased.

2. That a rather indefinite minimum 90 amount of oil (proportional to the weight of the minerals to be concentrated) must be used.

3. That, above a similar rather indefinite maximum amount, the additional oil is of no 95 advantage.

4. That a large excess of oil decreases the buoyancy of the oil-mineral-bubble floccules.

5. That the amount of oil used to secure 100 similar results with different ores is proportional to the weight of the concentrates.

6. That the amount of oil increases with the fineness of grinding and is somewhat different with different ores and different oils. 105

7. That the machines producing the largest amount of the finest bubbles give the best results.

8. That the concentrate can be "cleaned" 110 by successive treatments, the more fine bubbles present the better the cleaning.

9. That some of the fine silica can be washed out of the floccules after their removal and settlement in water.

10. That the finest part of the gangue- 115 material remains in the floccules.

The theory of the action of the metallic iron is as follows:

During the grinding operation (or during the abrasion of the iron by violet agitation of the pulp in the presence of the iron) minute particles of iron are rubbed off the grinding parts. As these particles are positively charged they are constantly attracted by the fine gangue particles and the finer gangue particles i. e. quartz and silicates are especially attracted by the iron particles which carry a relatively large charge. The very fine iron is quickly oxidized and, as the iron and gangue particles 120

125

130

135

are continually attracted to each other, a large part of this oxidation takes place when the iron and silica are in contact and results in the coating of the silica with a fine film of iron oxide. As the charge is entirely on the surface of a particle, these coated gangue particles are now positively charged and enter the floccules in the same way as the ore-minerals. This theory is borne out by the fact that the gangue-minerals which are rendered oil-flocculable by grinding or scouring with iron ore are in every case colored a tan color in the grinding or scouring process. The shade of this coloration will vary from a very faint tinge to a deep tan or brown, according to the time of contact or grinding, and the amount of iron surface exposed to scouring or grinding. The gangue-particles rendered oil-flocculable by this treatment with iron according to this theory should act in a manner similar to the ore minerals in every respect, not only in being oil-flocculated but also with respect to the effect of acids, alkalis and other electrolytes which is found to be the case in practical operation. The removal of this effect of the iron on the quartz and silicates by treatment with acid consists in the dissolving or removing of this thin iron oxide coating, and thus restoring these gangue minerals to their uncoated condition in which condition they are negatively charged.

The reason that the residual acid from this acid treatment should be neutralized with limestone rather than an alkali is that the iron oxide precipitated by the alkali tends to recoat the particles of quartz and silicates. It is also much easier to secure a neutral solution by using the limestone.

The theoretical explanation of the effect of fine metallic (unoxidized) iron (or other metal) in the pulp is that the metallic iron particles carry relatively very large positive charges. The metallic iron particles are wet by the oil and enter the floccules with the ore-minerals, thus giving the floccules a relatively very large positive charge. As the effect of this charge cannot be neutralized with air bubbles owing to the limited capacity of the floccules to hold these, the effect of this additionally large charge must be neutralized by the gangue-mineral particles, thus bringing more gangue mineral into the floccules. Theoretically this effect should be proportional to the amount of iron and would be small with very small amounts of iron. This is shown to be the case in all the tests made on this point as previously noted. This effect is very much smaller in practical operation than the previously described effect when the iron is oxidized and coats the gangue mineral particles. The theory of the action of the iron explains the very poor results secured in an iron machine. It also explains the slightly better

results secured in a non-metallic machine as compared with a metallic one, such as aluminum, as the violent agitation would scour off a small amount of very fine metal into the pulp, especially if the pulp contained much coarse material. The latter part explains the slightly poorer results on the aluminum machine.

According to the electrical theory, the minerals to be concentrated must be finely ground in order that the mass of each of the particles be not too large in proportion to its surface as the latter determines the amount of charge that the particles can carry. The fineness of grinding necessary should also vary with the different minerals according to the capacity of the surface of the particles of these to hold an electrical charge. Practical experience with the process is in strict accord with this theory, those minerals which have the greatest capacity for taking a charge requiring the least reduction in size. The minerals which have this capacity in a greater degree are those which are the most crystalline and whose cleavage faces come nearest to a metallic lustre. This is most strikingly borne out by the preferential action of the process on different ore-minerals, for example, with azurite and malachite.

According to the electrical theory only those oils would be useful in my process which are practically insoluble in water, and which can be broken up into minute globules in the water, and thus become charged. This is strikingly confirmed by considering the oils which are useful in the process, and explains the deleterious effect of soluble oils, which tend to dissolve the insoluble oils and make them more soluble. This also partially explains the fact that the essential oils are not useful in the process. These oils are partially soluble and do not break up into globules but surround the air bubbles and therefore act in an entirely different manner to the other types of oils, such as the fixed oils, and the rosin mixtures.

According to the electrical theory, the finer bubbles would be much more active in the process which is in strict accordance with practical results.

The theoretical explanation of the effect of acid is twofold. First, the acid discharges all the particles in the pulp, as in ordinary flocculation for settling or sedimentation, and thereby destroys any selective electrical attraction between the different constituents of the pulp. Second, the acid also tends to prevent the breaking up of the oil into minute globules, since as oil globules are discharged by the acid they flocculate, i. e., come together like other substances, but, instead of forming flocks like other substances, from large globules which would again tend to unite to form larger

globules due to the action of the surface tension of the oil. This latter effect is instantly shown when acid is added to water in which the oil has been dispersed. The dispersion is immediately destroyed and larger globules of oil formed.

The theory of the action of the alkali is also two-fold. First the alkali increases the charges on the particles and gives all the particles in the pulp the same kind of charge, greatly increasing the dispersion and entirely preventing any flocculation. Second, the alkali acts on and dissolves the oil making a soluble compound which prevents dispersion of the oil into globules of the character necessary in the process. The oil loses its power of dispersion into globules and instead coats the fine air bubbles in a manner similar to the essential oils forming a mass of white foam which has no action on the minerals in the deflocculated pulp. The action of soap which is alkaline is similar to that of the alkalis.

The theory of the action of the neutral electrolytes is that the addition of the salt first entirely discharges the mineral particles. The mass attraction between the particles then causes them to flocculate non-selectively. When the oil is added to a pulp in this condition, the non-selective flocks are first oil-flocculated as such, and this action is entirely non-selective. As it is only the mass attraction, which is relatively very weak, which holds the excess gangue particles in the oil-floccules, these particles are soon displaced by a vigorous agitation and remain in a relatively dispersed condition, as compared with the oil floccules, though in a flocculated condition, in the pulp. When the pulp becomes quiet these gangue particles settle out in flocks of the ordinary kind such as occur in ordinary settlement or sedimentation. This shows clearly that ordinary flocculation and the selective oil-flocculation of my process are entirely distinct and separate phenomena. According to this theory, only the neutral salts which flocculate the pulp would have the effect described. This is found to be the case, some electrolytes being helpful in the process.

According to the foregoing theory the fine particles of siliceous gangue-material remaining in the pulp after the removal of the concentrates should be left in a relatively highly dispersed condition as these particles are all negatively charged and tend to repel each other and remain dispersed. In practice this is found to be the case. The tailings solutions from the flotation cells remain milky for a considerable period, and it is practically impossible to settle or filter them without adding acid to discharge these negatively charged particles. The action of the fine particles of tailings is in

marked contrast to the quick settling of the finely ground ores which usually settle quite rapidly, but this is also in accord with the foregoing theory as, unless the particles of gangue and ore-mineral are kept in constant agitation (when there would be a constantly recurring charging and neutralizing of the ore and gangue-particles by each other) their opposite charges should neutralize each other, and the pulp should flocculate more or less rapidly and settle quickly. This is found to be the case in practice, the finely ground ores which contain the two classes of minerals in nearly equal proportions settle much more quickly than ores containing very unequal proportions of the two classes of minerals. The ores ground with iron also settle much more slowly than those ground with quartz pebbles, which should be the case according to the theory, since in the iron grinding operation the gangue particles are changed so as to all carry positive instead of negative charges, and therefore all the particles in the pulp being similarly charged should repel each other, remain dispersed, and settle slowly.

The theory of selective oiling of the ore-mineral particles is as follows: The wetting or oiling of the ore-mineral particles is not intrinsically due to the opposite charges of the particles of the two, since the gangue-mineral particles in the floccules have the same chance as the ore-minerals of being oiled. There is, however, a selective oiling of the ore-minerals in the presence of the gangue-minerals. At the root of this action is a chemical or quasi-chemical reaction or tendency to chemical action between an ingredient of the oil and the ore-minerals. That this is the case is indicated by the fact that only those oils which contain a fatty or rosin acid, or analogous compound are active in the process. The fatty acids do form compounds with the bases which (other than those with the alkalis) are relatively insoluble in water, but are relatively more soluble in the oil or oil compound. The theory of the selective oiling is then that the acid constituent of the oil acts superficially upon the surface of the ore-mineral, and either forms a compound which is more soluble in the oil than in water, or due to this chemical tendency causes the adsorption of the oil or a constituent thereof at the surface of these particles and thereby causes these minerals to be preferentially wet by the oil.

According to this theory, the minerals which are acted upon with difficulty by chemical reagents would not be oiled while those minerals which are easily acted upon by chemical reagents are oiled. This corresponds with the fact that the process is especially applied to the separation of the minerals which as a class are not acted upon

by ordinary chemical reagents, i. e., are relatively insoluble, from those which as a class are relatively easily acted upon by chemical reagents, i. e., are relatively soluble.

- 5 According to this theory, the oils would tend to wet only those minerals which contain a base with which the acid component of the ore could form a compound. This corresponds with the fact that no form of mineral composed of  $\text{SiO}_2$  is wet by the oil. According to this theory only those oils which would have a tendency to act chemically upon the ore-minerals would oil the ore-minerals which explains why the essential oils and mineral oils, which are neutral hydrocarbons, do not oil these minerals.

10 Also according to this theory, since this quasi-chemical reaction, chemical reaction or chemical tendency is relatively weak, its 20 effect is destroyed unless the conditions are favorable and therefore such strong factors as the effect of acids and alkalis destroy the operation of this force.

According to this theory the rapidity of 25 oiling should be different with different minerals, and the more insoluble should take the longer time for oiling. This is found to be the case in practice almost without exception, for example the few silicate ore 30 minerals, which are more or less insoluble, require a considerable period of mixing in order to be oiled and oil-flocculated. According to this theory there would be no sharp break between the two classes of minerals which are separated by my process but 35 the two classes would be joined by minerals having characteristics intermediate between the two as to solubility. As before noted this is found to be the case in testing out the 40 different minerals and ores.

From the foregoing it is readily seen that my process is not an entirely empirical process but is based upon a well substantiated scientific theory which is a valuable guide 45 to the investigation of each step in the process and to the investigation of the oils which can be used and the ores or minerals which can be treated, and makes possible the understanding of unusual phenomena occurring 50 in the practical operation of the process and suggests the remedies for the conditions which cause these phenomena.

This theory is a generalization drawn from a very large amount of research work 55 and observation extending over a considerable period of time, and is strikingly verified by all the phenomena of the practical operation of the process.

It is to be understood, however, that 60 while I believe the exposition of the theory as above outlined is correct, that I do not desire to be limited thereby, and the same is given merely to elucidate and make clear the very wide field of useful application which 65 is open to my process.

The great efficiency of my process is shown by the following reports on tests of a few widely different ores.

A manganese ore consisting mainly of manganeseite in a porphyry gangue:

70

|                   | % Weight. | % Mn. | % Insoluble. |
|-------------------|-----------|-------|--------------|
| Heads.....        | 100       | 30.1  |              |
| Concentrates..... | 47        | 60.3  |              |
| Tailings.....     | 53        | 3.8   | 5            |
| Recovery.....     |           | 94    |              |

High grade copper carbonate ore in sandstone:

80

|                   | % Weight. | % Cu. | % $\text{SiO}_2$ . |
|-------------------|-----------|-------|--------------------|
| Heads.....        | 100       | 12.3  | 76                 |
| Concentrates..... | 27        | 45.6  | 13.2               |
| Tailings.....     | 73        | 0.3   | 96.8               |
| Recovery.....     |           | 98.0  | 85                 |

Oxidized lead ore in silicified limestone:

Assay.

90

|                   | % Wt. | Oz. Au. | Oz. Ag. | % Pb. | % Cu. | % CaO. | % Fe. | % $\text{SiO}_2$ . |
|-------------------|-------|---------|---------|-------|-------|--------|-------|--------------------|
| Heads.....        | 100   | .025    | 17.2    | 11.8  | .1    | 4.6    | 3.3   | 65.6               |
| Concentrates..... | 35    | .07     | 45.3    | 32.6  | .3    | 11.5   | 7.9   | 12.2               |
| Tailings.....     | 65    | Trace.  | 2.2     | .2    | Tr.   | .8     | .5    | 95.1               |
| Recovery.....     |       | 95      | 91.5    | 96.6  | 95    | 89.7   | 83.8  | .....              |

Low grade copper carbonate ore in sandstone:

100

|                   | % Wt. | % Cu. | % $\text{SiO}_2$ . |
|-------------------|-------|-------|--------------------|
| Head.....         | 100   | 2.1   |                    |
| Concentrates..... | 5.1   | 38.6  | 31                 |
| Middlings.....    | 6     | 2.4   | 82.9               |
| Tailings.....     | 88.9  | .10   | 96.1               |
| Recovery.....     |       | 94    | .....              |

105

A large number of tests on many different kinds of ores show results of the same character as the foregoing. Oxidized ores of copper, lead, zinc, manganese and ores carrying oxidized minerals of value such as carnotite, etc., in different siliceous gangues are amenable to treatment with excellent results. As it is obviously impossible to give the many small variations possible in the commercial application of my process in the scope of a patent application I desire to be limited only by the appended claims as interpreted in the light of the foregoing specifications.

110

This application is a continuation in part of my application Serial No. 230,792, filed as of April 25, 1918.

115

What is claimed is:

120

1. The art of concentrating natural oxidized ores, i. e. unaltered except by grinding, which consists in forming with such oxidized ores in comminuted form an aqueous pulp free from electrolytes which inhibit the selective formation of oil-mineral floccules

130

- containing non-siliceous minerals, adding an oily substance, substantially insoluble in water, containing an organic acid radical in proportion to form oil-mineral floccules in which the non-siliceous minerals of the ore are concentrated, agitating the said mixture and separating the floccules thereby formed from the remainder of the pulp containing the siliceous minerals of the ore.
2. The art of concentrating natural oxidized ores, i. e. unaltered except by grinding, which consists in forming with such oxidized ores in comminuted form an aqueous pulp free from electrolytes which inhibit the selective formation of oil-mineral floccules containing non-siliceous minerals, adding an oily substance, substantially insoluble in water, containing an organic acid radical in proportion to form oil-mineral floccules in which the non-siliceous minerals of the ore are concentrated, agitating the said mixture and separating the floccules thereby formed from the remainder of the pulp containing the siliceous minerals of the ore by flotation.
3. The art of concentrating natural oxidized ores, i. e. unaltered except by grinding, which consists in forming with such oxidized ores in comminuted form an aqueous pulp free from electrolytes which inhibit the selective formation of oil-mineral floccules containing non-siliceous minerals, adding an oily substance, substantially insoluble in water, containing an organic acid radical in proportion to form oil-mineral-floccules in which the non-siliceous minerals of the ore are concentrated, agitating and aerating the said mixture whereby the non-siliceous minerals are selectively oiled and forming a buoyant flocculent froth and separating the froth thereby formed from the remainder of the pulp containing the siliceous minerals of the ore.
4. The art of concentrating natural oxidized ores, i. e. unaltered except by grinding, which consists in forming with such oxidized ores in comminuted form an aqueous pulp free from electrolytes which inhibit the selective formation of oil-mineral floccules containing non-siliceous minerals, adding an oily substance, substantially insoluble in water, containing an organic acid radical in proportion to form oil-mineral-floccules in which the non-siliceous minerals of the ore are concentrated, agitating the said mixture substantially without contact with metallic iron and separating the floccules thereby formed from the remainder of the pulp containing the siliceous minerals of the ore.
5. The process of treating oxidized ores as such, i. e. unaltered otherwise than by grinding, which consists in finely grinding the ore with siliceous grinding media, forming with the finely ground ore an aqueous pulp free from electrolytes which inhibit the selective formation of oil mineral floccules containing non-siliceous minerals, adding an oily agent, substantially insoluble in water, containing an organic acid radical in proportion to form oil-mineral floccules in which the non-siliceous minerals of the ore are concentrated, and agitating said mixture and separating the floccules thus formed from the residue of pulp containing the siliceous minerals of the ore.
6. The process of treating oxidized ores, as such, i. e. unaltered otherwise than by grinding, which consists in finely grinding the ore with siliceous grinding media, forming with the finely ground ore an aqueous pulp free from electrolytes which inhibit the selective formation of oil mineral floccules containing non-siliceous minerals, adding an oily agent substantially insoluble in water; containing an organic acid radical in proportion to form oil-mineral floccules in which the non-siliceous minerals of the ore are concentrated, and agitating and aerating said mixture whereby the non-siliceous minerals are selectively oiled and form a buoyant flocculent froth and separating the froth thus formed from the residue of pulp containing the siliceous minerals of the ore.
7. The process of treating oxidized ores as such, i. e. unaltered otherwise than by grinding, which consists in finely grinding the ore with siliceous grinding media, forming with the finely ground ore an aqueous pulp free from electrolytes which inhibit the selective formation of oil mineral floccules containing non-siliceous minerals, adding an oily agent substantially insoluble in water, containing an organic acid radical in proportion to form oil-mineral floccules in which the non-siliceous minerals of the ore are concentrated, and agitating and aerating said mixture substantially without contact with metallic iron whereby the non-siliceous minerals are selectively oiled and form a buoyant flocculent froth and separating the froth thus formed from the residue of pulp containing the siliceous minerals of the ore.
8. The process of treating oxidized ores as such, i. e. unaltered otherwise than by grinding, which consists in finely grinding the ore with siliceous grinding media, forming with the comminuted ore an aqueous pulp free from electrolytes which inhibit the selective formation of oil-mineral floccules containing non-siliceous minerals, adding an oily agent, substantially insoluble in water, containing an organic acid radical, in a proportion equal to approximately ten to fifteen per cent of the weight of the non-siliceous minerals of the ore, and agitating and aerating said mixture whereby the non-siliceous minerals are selectively oiled and form a buoyant flocculent froth, and separating said froth from the remainder of the pulp containing the siliceous gangue minerals of the ore.

9. The process of treating oxidized ores as such, i. e. unaltered otherwise than by grinding, which consists in finely grinding the ore with siliceous grinding media, forming with the comminuted ore an aqueous pulp free from electrolytes which inhibit the selective formation of oil-mineral floccules substantially insoluble in water, containing non-siliceous minerals, adding an oily agent, 5 containing an organic acid radical, in a proportion equal to approximately ten to fifteen per cent of the weight of the non-siliceous minerals of the ore, and agitating and aerating said mixture substantially without contact with metallic iron whereby the non-siliceous minerals are selectively oiled and form a buoyant flocculent froth, and separating said froth from the remainder of the pulp containing the siliceous gangue minerals of the ore. 10
10. The process of treating oxidized ores as such, i. e. unaltered otherwise than by grinding, which consists in finely grinding the ore with siliceous grinding media, forming with the comminuted ore a neutral aqueous pulp, mixing with said pulp an oily agent which will selectively oil the non-siliceous minerals in a proportion approximately ten to fifteen per cent of the weight 15 of the non-siliceous minerals of the ore, and agitating and aerating said mixture whereby the non-siliceous minerals are selectively oiled and concentrated into buoyant flocculent froth, and separating said froth from the remainder of the pulp containing the siliceous gangue minerals of the ore. 20
11. The process of treating oxidized ores as such, i. e. unaltered otherwise than by grinding, which consists in finely grinding the ore with siliceous grinding media, forming with the comminuted ore a neutral aqueous pulp, mixing with said pulp an oily agent which will selectively oil the non-siliceous minerals in a proportion approximately ten to fifteen per cent of the weight 25 of the non-siliceous minerals of the ore, and agitating and aerating said mixture substantially without contact with metallic iron whereby the non-siliceous minerals are selectively oiled and concentrated into buoyant flocculent froth, and separating the froth thus formed from the residue of pulp containing the siliceous minerals of the ore. 30
12. The process of treating oxidized ores as such, i. e. unaltered otherwise than by grinding, which consists in finely grinding substantially without contact with metallic iron, forming with the finely ground ore an aqueous pulp free from electrolytes which inhibit the selective formation of oil-mineral floccules containing non-siliceous minerals, adding an oily agent substantially insoluble in water containing an organic acid radical; in proportion to form oil-mineral floccules in which the non-siliceous minerals 35 of the ore are concentrated, and agitating and aerating said mixture whereby the non-siliceous minerals are selectively oiled and form a buoyant flocculent froth, and separating the froth thus formed from the residue of pulp containing the siliceous minerals of the ore. 40
13. The process of treating oxidized ores as such, i. e. unaltered otherwise than by grinding, which consists in finely grinding substantially without contact with metallic iron, forming with the finely ground ore an aqueous pulp free from electrolytes which inhibit the selective formation of oil mineral floccules containing non-siliceous minerals, adding an oily agent, substantially insoluble in water containing an organic acid radical in proportion to form oil-mineral floccules in which the non-siliceous minerals of the ore are concentrated, and agitating and aerating said mixture whereby the non-siliceous minerals are selectively oiled and form a buoyant flocculent froth and separating the froth thus formed from the residue of pulp containing the siliceous minerals of the ore. 45
14. The process of treating oxidized ores as such, i. e. unaltered otherwise than by grinding, which consists in finely grinding substantially without contact with metallic iron, forming with the finely ground ore an aqueous pulp free from electrolytes which inhibit the selective formation of oil-mineral floccules containing non-siliceous minerals, adding an oily agent substantially insoluble in water, containing an organic acid radical in proportion to form oil-mineral floccules in which the non-siliceous minerals of the ore are concentrated, and agitating and aerating said mixture substantially without contact with metallic iron whereby the non-siliceous minerals are selectively oiled and form a buoyant flocculent froth and separating the froth thus formed from the residue of pulp containing the siliceous minerals of the ore. 50
15. The process of treating oxidized ores as such, i. e. unaltered otherwise than by grinding, which consists in finely grinding substantially without contact with metallic iron, forming with the comminuted ore an aqueous pulp free from electrolytes which inhibit the selective formation of oil-mineral floccules containing non-siliceous minerals, adding an oily agent, substantially insoluble in water containing an organic acid radical, in a proportion equal to approximately ten to fifteen per cent of the weight of the nonsiliceous minerals of the ore, and agitating and aerating said mixture whereby the non-siliceous minerals are selectively oiled and form a buoyant flocculent froth, and separating said froth from the remainder of the pulp containing the siliceous gangue minerals of the ore. 55
16. The process of treating oxidized ores as such, i. e. unaltered otherwise than by grinding, which consists in finely grinding 60

substantially without contact with metallic iron, forming with the comminuted ore an aqueous pulp free from electrolytes which inhibit the selective formation of oil-mineral floccules containing non-siliceous minerals, adding an oily agent, substantially insoluble in water containing an organic acid radical, in a proportion equal to approximately ten to fifteen per cent of the weight 10 of the non-siliceous minerals of the ore, and agitating and aerating said mixture substantially without contact with metallic iron whereby the non-siliceous minerals are selectively oiled and form a buoyant flocculent froth, and separating said froth from the remainder of the pulp containing the siliceous gangue minerals of the ore.

17. The process of treating oxidized ores as such, i. e. unaltered otherwise than by 20 grinding, which consists in finely grinding substantially without contact with metallic iron, forming with the comminuted ore a neutral aqueous pulp, mixing with said pulp an oily agent which will selectively oil the 25 non-siliceous minerals in a proportion approximately ten to fifteen per cent of the weight of the non-siliceous minerals of the ore, and agitating and aerating said mixture whereby the non-siliceous minerals are 30 selectively oiled and concentrated into buoyant flocculent froth, and separating said froth from the remainder of the pulp containing the siliceous gangue minerals of the ore.

35 18. The process of treating oxidized ores as such, i. e. unaltered otherwise than by grinding, which consists in finely grinding substantially without contact with metallic iron, forming with the comminuted ore a neutral aqueous pulp, mixing with said pulp an oily agent which will selectively oil the non-siliceous minerals in a proportion approximately ten to fifteen per cent of the weight 40 of the non-siliceous minerals of the ore, and agitating and aerating said mixture substantially without contact with metallic iron whereby the non-siliceous minerals are selectively oiled and concentrated into buoyant flocculent froth, and separating said 45 froth from the remainder of the pulp containing the siliceous gangue minerals of the ore.

50 19. The process of treating oxidized ores, as such, which consists in finely grinding the ore out of contact with metallic iron media, forming with the finely ground ore an aqueous pulp free from electrolytes which inhibit the selective formation of oil floccules containing non-siliceous minerals, 55 mixing with said pulp an oily agent which will selectively oil the non-silicate minerals and leave the siliceous gangue minerals un-oiled, and agitating said mixture, and dur-

ing the production and treatment of the pulp maintaining the same out of contact with metallic iron surfaces whereby the non-silicate minerals are selectively oiled and form a buoyant flocculent froth, and separating said froth from the remainder of the pulp containing the siliceous gangue minerals. 70

20. The process of treating oxidized ores as such, i. e. unaltered otherwise than by grinding, which consists in finely grinding the ore with siliceous grinding media, forming with the finely ground ore a neutral 75 aqueous pulp containing in solution no acids, alkalis, acid salts or alkaline salts, in sufficient quantity to give any other than a neutral reaction to the pulp, mixing with said pulp an oily agent which will selectively oil the non-siliceous mineral particles and will leave the siliceous minerals unoiled, and agitating and aerating said mixture without sufficient contact with metallic iron to destroy the selective action of the oil, whereby the non-siliceous minerals are selectively 80 oiled and form a buoyant flocculent froth, and separating said froth from the remainder of the pulp containing the siliceous gangue mineral particles of the ore. 85

21. The process of treating oxidized ores as such, i. e., unaltered otherwise than by grinding, which consists in finely grinding the ore with siliceous grinding media, forming with the finely ground ore a neutral 95 aqueous pulp, mixing with said pulp an oily agent which will selectively oil the non-silicate minerals and leave the siliceous gangue minerals unoiled, and agitating and aerating said mixture without appreciable contact with metallic iron, whereby the non-silicate minerals are selectively oiled and form a buoyant flocculent froth, and separating said froth from the remainder of the pulp containing the siliceous gangue minerals. 100

22. The process of treating oxidized ores, as such, which consists in finely grinding the ore out of contact with metallic iron media; forming with the finely ground ore a neutral aqueous pulp; mixing with said pulp an oily agent which will selectively oil the non-silicate minerals and leave the siliceous gangue minerals unoiled; and agitating and aerating said mixture, and during the production and treatment of the pulp maintaining the same out of contact with metallic iron surfaces, whereby the nonsilicate minerals are selectively oiled and form a buoyant flocculent froth; and finally separating said froth from the remainder of the pulp 115 containing the siliceous gangue minerals. 120

In testimony whereof I have signed my name to this specification.

NIELS C. CHRISTENSEN.

Witness:

THEODORE STEBBINS.